

## UNITED STATES PATENT OFFICE

1,960,176

PROCESS OF MAKING AND UTILIZING  
SHEETED ADHESIVES AND THE PROD-  
UCTS THUS PRODUCEDJosef Weber and Franz Hengstebeck, Essen-  
Ruhr, Germany, assignors, by mesne assign-  
ments, to Th. Goldschmidt Corporation, New  
York, N. Y., a corporation of DelawareNo Drawing. Application June 2, 1931, Serial No.  
541,734. In Germany February 2, 1929

7 Claims. (Cl. 91—68)

This invention relates to processes of making and utilizing sheeted adhesives and to products thus obtained; and it comprises as a new adhesive article a substantially dry, substantially homogeneous, thin flexible sheet of an alkaline condensation product of formaldehyde with a phenol, said sheet ordinarily containing a tenuous fiber reinforcement and said product being solid at ordinary temperature, becoming plastic and melting when warmed and setting to a hard permanent infusible form at temperatures somewhat above 100° C.; and it also comprises processes of making said adhesive articles and it further comprises methods of utilizing said new adhesive article and products so obtained; all as more fully hereinafter set forth and as claimed.

In the usual method of cementing wood to wood, including affixing veneers and making plywood, the surfaces are treated with a solution of glue and setting performed under heat and pressure. Setting is really a removal of water and where extensive surfaces are united, the water is taken up by the wood. Most liquid glues contain large proportions of water and in making plywood, the amount of water to be dissipated in the glue used may be as high as 30 to 40 per cent of the weight of the wood to be joined. In building up plywood assemblages, the glue is applied to inner layers and the water is taken up by proximate layers thereby necessarily swelling these. At this stage in the operation the product includes a swollen inner wood layer connected to less moist outer layers or plies. In drying, the swollen inner layers tend to shrink to their original proportions thereby setting up heavy stresses and causing warping. Making plywood in this manner by the assemblage of successive laminae of wood with intermediate drying is a tedious operation and the product is apt to be irregular. The whole assemblage must be finally dried and unless this final drying, as well as the intermediate dryings, be conducted with exceptional care and skill an unsatisfactory product results. It may be warped, mottled or exhibit fissures (incipient cleavage). In order to obviate these difficulties it has been proposed to manufacture plywood and affix veneers by employing between the layers of wood a cementing layer in the form of glue-surfaced sheets of paper, of fabric, or even of wood. In making the cementing layer, suitable sheets are passed through a glue solution and afterwards dried so as to form adhesive surfaced sheets adapted to be interposed between the wood plies. Using sheets of this character the amount of wa- ter necessary can be limited to that required to

make the surface of the sheets sticky; and this is an advantage. This method while better than the more common procedure of cementing by liquid glue directly applied is nevertheless open to certain objections. For one thing in the final product, there is an intermediate structural element between the wood plies. For another, plywood made in this manner when subjected to changes in temperature and moisture conditions frequently tends to split apart along the plane of the intermediate fabric layer; the layer carrying the glue on its surfaces. Unless the glue is water-proofed in some manner, the dried layer is not resistant to the action of moisture.

In affixing veneers and in making plywood it is desirable to have the wood layers as close together, face to face, as possible, restricting the amount of intermediate adhesive to that sufficient to even out surface irregularities. And it is desirable to have an adhesive requiring in setting the dissipation of no great amount of water or of a volatile solvent; of any amount causing substantial swelling in the wood. These results are accomplished in the present invention where in is provided a thin substantially dry, substantially homogeneous lamina of adhesive usually containing a tenuous fiber reinforcement in negligible amount; the adhesive being solid at the ordinary temperature, softening and fusing to a mobile liquid at higher temperatures and finally setting to a hard infusible, permanent form on exposure to temperatures such as are used in making plywood, say at 130° C.

For our purpose we use a particular condensation product of a phenol and formaldehyde in the presence of a rather large amount of alkali; this alkali serving both as a catalyst in inducing condensation and having certain other functions. As the phenol, ordinary phenol may be used or one of the cresols. In lieu of formaldehyde, acetaldehyde or other aldehydes may be employed. However, ordinary phenol and ordinary formaldehyde, as the commercial 40 per cent solution, give good results. On dissolving equivalent amounts of phenol and formaldehyde (in solution) in 40 per cent caustic soda lye using the amount of lye necessary for solution, a satisfactory preparation can be made for the present purposes. With a batch of 94 kilograms of phenol and 100 kilograms of commercial 30 per cent formaldehyde solution about 17 kilograms of 40 per cent NaOH solution give a good preparation. This liquid is kept warm for a time say at 80° C. for 1½ hours, with constant stirring until an easy flowing oily dark liquid is obtained.

Heating must be stopped before an aqueous layer separates from the reaction products. The separation of such a layer shows that the reaction has gone too far and the condensation product obtained will not possess the advantageous properties here desired. The viscosity of the product obtained depends upon the time of heating but is rather low in any event. The exact viscosity desired can be obtained by interrupting the heating and then cooling. Because of the solvent influence of the excess of alkali and of the water present, no separation into two layers is produced. The oily liquid can be dried to a substantially dry material at temperatures below about 100° C. without going into the final insoluble resin. Ordinarily it is desired to dry the material to about 2 per cent water. By proper manipulation the dried material may be made in thin sheets. These sheets at the ordinary temperature are not tacky but are somewhat hygroscopic in the sense that they will take up more water from the air. Ordinarily the amount taken up will give a final product of about 5 to 8 per cent; this varying with the humidity. With this content of water the product is flexible and not sticky or tacky and the sheets can be packaged, shipped and stored as rolls without danger of adhesion.

As so far described, the sheets are made without the use of a reinforcement but for manufacturing reasons it is better to employ a tenuous reinforcement of fiber in negligible amount; an amount insufficient to produce a substantial intervening layer between the sheets of wood ultimately to be united. As this reinforcement we employ an open textured, thin paper, or like sheeted material. With the aid of this paper it is possible to produce the present material by ordinary manufacturing operation in a continuous manner; a web of paper passing first through the initial condensation product, past equalizing rolls and then through drying apparatus. Drying is usually so conducted as to give about 2 per cent water in the dry material and sufficient exposure to air is then permitted to allow assumption of the full amount of "water of condition"; usually about 8 per cent. The proportion of fiber to adhesive varies but is usually in about the ratio of 1 : 2. With thin open textured paper in this proportion the final sheeted product has a substantially continuous body of adhesive. In making such completely and uniformly impregnated sheets which are in fact continuous films of adhesive, the thickness and porosity or open texture of the reinforcing sheet are so correlated with the liquidity or viscosity of the oily liquid condensation product containing caustic soda as to insure a complete, continuous and uniform impregnation. When this relation is properly established the oily liquid penetrates all the pores of the reinforcing medium and it is only necessary to apply the proper amount of liquid to give the desired ratio of condensation product to the reinforcing material.

The presence of the caustic soda (for which caustic potash may be substituted), in the composition in about the amount indicated gives a preparation which at the ordinary temperature is not tacky; is not hygroscopic enough to become moist and sticky in ordinary air. It does however take up a little water of condition; enough to make it flexible and easily handled. The dry composition on warming to a few degrees above the ordinary temperature becomes plastic

enough to facilitate easy sheeting and on recooling is permanent; it can be stored, packaged and handled without trouble. In heating to fusion in use, probably the caustic soda and the small amount of water of condition present exercise a solvent action or contribute to fusion. The caustic soda solution produces condensation in making the initial oily liquid but it does not cause condensation much beyond this point with any reasonable degree of temperature until the heat reaches a point somewhere around 130° C. when the catalytic action becomes extremely rapid. In the final product the caustic soda does not exist in any form making the article hygroscopic; nor is it necessary in making plywood to provide for the dissipation of the water present in the mixture. It is, in any event, small in amount being only about 5 to 8 per cent of the adhesive.

When the flexible sheeted adhesive (with or without reinforcement) is placed between two layers of wood in the usual way of affixing veneers or making plywood and heat and pressure are applied, the adhesive at first yields and softens, then fuses and is then taken up for the most part by the pores of the wood; finally solidifying in place. With about 8 per cent water in the material on fusing it forms a fairly mobile liquid readily taken up by pores as a whole; there being no segregation of solvent by the pores of the wood as there usually is with moist glue made plastic by heat. The alkali and water have a fluxing action but the melt is homogeneous. In the presence of the alkali and water, there is some reaction on the wood fiber contributing to the extremely perfect cohesive union ultimately secured.

On heating the assemblage of plies and adhesives up to, say, 130° C. the condensation products are converted into the final insoluble resin without much change in volume and with very little extrication of water; not enough to cause swelling or require any special care in subsequent drying.

Because of the properties of the present adhesive sheet it is possible to join a number of layers of plywood together simultaneously instead of successively as is the usual practice; thereby economizing time and labor.

While the invention has been particularly described in its use in cementing veneers and making plywood, the adhesive sheets of the present invention are advantageous in many other relations and may be used for general cementing purpose. Their use in forming a facing layer on various articles is advantageous.

What we claim is:

1. As a new product, adhesive papers for plywood manufacture comprising a porous open textured tissue paper sheet impregnated with an initial condensation product of an aldehyde with a phenol, said condensation product containing a substantial amount of alkali, being capable of softening and fusing under heat and pressure to give a mobile liquid, being capable of hardening under said heat and pressure to give a hardened insoluble body, and having been produced at low temperatures in a dilute caustic alkali solution without separation of an aqueous layer.

2. As a new product, adhesive papers for plywood manufacture comprising a porous open textured thin tissue paper sheet impregnated with a low temperature, initial condensation product of an aldehyde with a phenol, caustic soda, and a small amount of water fixed as water of condition, said water being about 8 per cent of the total

80

90

95

100

105

110

115

120

130

135

140

145

150

adhesive, the ratio of said condensation product to the paper being about 2:1.

3. A process of making adhesive papers for plywood manufacture which comprises heating 5 formaldehyde with a phenol in an aqueous solution of caustic alkali under conditions suitable for producing a homogeneous, easy flowing, oily initial condensation product without the separation of an aqueous layer, impregnating a porous, open 10 textured tissue paper sheet with said product without the presence of extraneous solvents and drying to produce a non-tacky surface.

4. In the making of adhesive papers for plywood manufacture, the process which comprises 15 warming a phenol and formaldehyde together in the presence of an aqueous caustic soda solution under conditions suitable for producing a homogeneous oily, liquid condensation product without the separation of an aqueous layer, and impregnating a porous, open textured, thin tissue 20 paper sheet with said product and drying the impregnated paper, the amount of alkali present not being sufficient to give the dried sheet a tacky surface but being sufficient to cause absorption 25 of from about 5 to 8 percent of water of condition on exposure to air.

5. In the making of adhesive papers for plywood manufacture, the process which comprises reacting together an aldehyde and a phenol in 30 an aqueous solution of caustic alkali under conditions suitable for producing a homogeneous, oily, liquid, initial condensation product without separation of an aqueous layer, impregnating a porous, thin tissue paper sheet with said product and drying the impregnated sheet at temperatures 35 below about 100° C. to form a substantially dry, solid but flexible sheet containing a substantial amount of caustic soda and water of condition; the impregnating condensation product be-

ing capable of assuming a highly fluid state under heat and pressure at temperatures not substantially above 130° C.

6. As a new product, an adhesive sheet for plywood manufacture comprising a porous, open textured, tissue paper sheet impregnated with an initial condensation product of an aldehyde with a phenol, formed without separation of an aqueous layer and in the presence of a caustic soda solution, and containing a small amount of water fixed as a water of condition, said water being about 5 to 8 per cent of the total adhesive; the said condensation product being free from extraneous solvents, being capable of assuming a highly fluid state under heat and pressure at temperatures not substantially above 130° C. and, when placed between sheets of plywood and subjected to heat and pressure, being capable of fusing to form a mobile liquid and then hardening in situ to unite said sheets with a hard, insoluble bond.

7. As a new product an adhesive sheet for plywood manufacture comprising a porous, open textured, thin tissue paper sheet impregnated with a low-temperature, initial condensation product of an aldehyde with a phenol formed in the presence of a caustic alkali solution, the said condensation product being free from extraneous solvents, being capable of assuming a highly fluid state under heat and pressure at temperatures not substantially above 130° C. and, when placed between sheets of plywood and subjected to heat and pressure, being capable of fusing to form a mobile liquid and then hardening in situ to unite said sheets with a hard, insoluble bond.

JOSEF WEBER.  
FRANZ HENGSTEBECK.

40

115

45

120

50

125

55

130

60

135

65

140

70

145

75

150